

Feb. 24, 1931.

R. K. PAINTER

1,793,957

METHOD AND APPARATUS FOR EMULSIFYING ASPHALT

Filed Feb. 1, 1930



INVENTOR.  
ROBERT K. PAINTER  
BY *B. Fraig*  
ATTORNEY.

## UNITED STATES PATENT OFFICE

ROBERT K. PAINTER, OF LOS ANGELES, CALIFORNIA, ASSIGNOR TO BITUTECT, INCORPORATED, OF LOS ANGELES, CALIFORNIA, A CORPORATION OF CALIFORNIA

## METHOD AND APPARATUS FOR EMULSIFYING ASPHALT

Application filed February 1, 1930. Serial No. 425,341.

This invention relates to a method and to an apparatus for emulsifying asphalt.

The general object of the invention is to provide an improved method and apparatus 5 for emulsifying bituminous substances.

One of the specific objects of the invention is to provide a novel method of producing asphalt emulsions.

A specific object of the invention is to provide 10 an improved method for emulsifying asphalt wherein the asphalt is first placed in solution.

An additional object of the invention is to provide 15 a method of emulsifying asphalt wherein the asphalt is first dissolved in a solvent after which a colloidal solution is added thereto and wherein the asphalt is thereafter precipitated in the presence of the colloidal solution by reaction with a suitable 20 re-agent.

A further object of the invention is to provide 25 a method of emulsifying asphalt or vegetable pitches wherein the asphalt or pitch is first dissolved in a solvent after which a colloidal solution is added thereto, and wherein the asphalt is thereafter precipitated 30 in the presence of the colloidal solution by reaction with a suitable re-agent after correcting the alkalinity of both by an addition of an aqueous solution of an organic acid to a degree whereby I will secure a superior stabilization, and whereby I may use smaller 35 percentages of mineral protective colloid than has been heretofore consistent with permanency of suspension.

A further object of the invention is to provide 40 an improved apparatus which is particularly adapted for emulsifying asphalt.

Other objects of the invention will be apparent 45 from the following description taken in connection with the accompanying drawings wherein:

Fig. 1 is a side elevation partly in section showing 50 an apparatus embodying the features of my invention, and

Fig. 2 is an enlarged view showing an emulsifier which may be used in connection with my invention.

Referring to the drawing by reference 55 characters, I have shown an asphalt storage

tank at 10. This tank is supported on suitable standards 11. The tank 10 is connected by a pipe 12 with a measuring tank 14. This measuring tank is in turn connected by a pipe 15 with an emulsifier 16. Suitable valves 17 55 and 18 are provided so that the measuring tank 14 may be utilized.

A mixing tank is shown at 19. In this mixing tank I place ingredients to make an aqueous solution of colloidal clay. This tank 60 19 is connected by a pipe 20 with a measuring tank 21. A pump 22 serves to force the colloidal solution through the pipe 20. This pump 22 may be driven by belts 23, 23' and 23'' from a motor 24 or it may be driven in 65 any other desired manner. The tank 21 is connected by means of a pipe 25 with the emulsifier 16. Valves 26 and 27 are arranged so that the measuring tank 21 may be operated. 70

The delivery pipe 28 from the emulsifier is controlled by a valve 29 and delivers into a product storage tank 30. The material in the product storage tank 30 may be removed 75 through the pipe 31 which is connected to a pump 32 and this pump delivers to a discharge pipe 33.

The emulsifier per se forms no part of my present invention but may be made of any 80 type. In the drawing it is shown as comprising a case having a steam jacket 34 thereabouts. Steam is supplied to the jacket through a pipe 35 while exhaust steam passes through a pipe 36.

This jacket serves to keep the mixture in 85 the emulsifier at the proper temperature.

The emulsifier is shown as provided with a beater 37 which may be driven by a shaft 38 which in turn is driven by cased gears 38' 90 from a shaft 38'': The shaft 38'' is driven from the belt 38a. The emulsifier is provided with a cover 39 which serves to prevent the escape of fumes.

I will now proceed to describe my improved method. As one example of this 95 method, I may dissolve asphalt of any desired grade or I may dissolve other bituminous substances and vegetable pitches in carbon tetrachloride or other suitable solvents. The solvent used is preferably vola- 100

tile. To the saturated solution thus formed I add preferably 30% of its volume of a colloidal solution such as an aqueous solution of colloidal clay. This aqueous solution of colloidal clay is preferably of a density of one pound of clay to one gallon of water. The vessel is preferably covered to prevent the escape of fumes, or to collect the fumes for condensation and re-use.

- 10 The temperature is raised to 130 degrees Fahrenheit. This done I add methyl acetone in sufficient quantities to effect precipitation. While the precipitation is going on I run the clay solution into the mixer. Melted asphalt 15 or other melted bitumen is also simultaneously added in the ratio of 2½ parts of asphalt or bitumen to one part of clay solution. The addition of the solution of clay and melted bitumen or asphalt is continued 20 indefinitely with a stabilizer comprising an aqueous solution of an organic acid such as citric, acetic, malic or oxalic acid, in the instance here given as an embodiment of my invention  $\frac{1}{16}$  of 1% by volume of a  $\frac{1}{16}$ <sup>N</sup> solution of 80% acetic acid, and the resultant emulsified asphalt or bitumen is drawn off. The proportions mentioned, it will be understood, serve as an example only and other proportions and other re- 25 agents may be employed if desired.

It is a well recognized fact that when asphalt or other material is precipitated chemically from solution that the particles are extremely fine. With my method the fine 30 comminution of the bitumen gives a superior product over that obtained by other methods.

Having thus described my invention, I claim:

1. The method of emulsifying asphalt 40 comprising first dissolving the asphalt in a solvent, adding to the solution thus formed an aqueous solution of colloidal clay of which the solid content is less than 2% of the emulsion produced, agitating the mixture at a de- 45 sired temperature, maintaining a desired true acidity by control with additions at this point of aqueous solution of an organic acid, precipitating the asphalt in the presence of said colloidal solution and at the 50 proper degree of true acidity while the whole is agitated.

2. The method of emulsifying asphalt comprising dissolving the asphalt in a suitable solvent, mixing the solvent with a colloidal solution and precipitating the asphalt in the presence of the colloidal solution at the proper true acidity, thereafter continuing the process by the addition of clay solution corrected with an organic acid and the 60 addition of melted asphalt and drawing off the product.

3. The method of emulsifying asphalt comprising first dissolving the asphalt in a solvent, adding to the saturated solution 65 thus formed an aqueous solution of colloidal

clay corrected as to acidity with an organic acid, agitating the mixture at a desired temperature, precipitating the asphalt by methyl acetone in the presence of said colloidal solution while the whole is agitated.

4. The method of emulsifying bituminous substances comprising first dissolving the bitumen in a solvent, adding to the solution thus formed a colloidal solution, precipitating the bitumen in the presence of said colloidal solution while the whole is agitated, thereafter continuing the process by the addition of clay solution, corrected as to acidity with an organic acid and melted asphalt introduced in thin streams and drawing off the product.

5. The method of emulsifying asphalt comprising first dissolving the asphalt in a volatile solvent, adding to the saturated solution thus formed, an aqueous solution of colloidal clay, agitating the mixture at a desired temperature, precipitating the asphalt by methyl acetone in the presence of said colloidal solution while the whole is agitated, thereafter continuing the process by the addition of clay solution, corrected as to acidity with an organic acid and melted asphalt introduced in thin streams and drawing off the product.

In testimony whereof, I hereunto affix my signature.

ROBERT K. PAINTER.

100

105

110

115

120

125

130